

## UNITED STATES PATENT OFFICE

2,315,135

## TEXTILE TREATING PROCESS

John B. Rust, Verona, N. J., assignor to Ellis-Foster Company, a corporation of New Jersey

No Drawing. Application May 5, 1942,  
Serial No. 441,811

5 Claims. (Cl. 117—167)

The present invention relates to a process of making water repellent textiles. An aim of the invention is to employ the water soluble reaction products described in my copending application Serial Number 392,937, filed May 10, 1941, now Patent No. 2,285,948, granted June 9, 1942. These products are formed by heating together a fatty acid nitrile containing a carbon chain of more than 9 carbon atoms with a fatty acid chloride containing a carbon chain of more than 9 carbon atoms and paraformaldehyde followed by reaction with a tertiary amine.

It has been found that by impregnating a textile fabric such as cotton, linen, viscose, acetate, wool or silk with a solution of the above described reaction products, thereafter drying the impregnated fabric and heating at an elevated temperature excellent water repellent characteristics are imparted to the fabric. By carrying out this process the product becomes fixed upon the fabric to such an extent that it is fast to washing and dry cleaning. In contrast with present known processes involving the development of water repellency by heating a fabric in the presence of compounds such as quaternary ammonium compounds, the present process does not result in a serious decrease in tensile strength of the fabric.

A fabric being so treated cannot be described as waterproof since it will readily wet out in warm water or cold water containing a wetting agent. However, when the fabric is dry it strongly repels water impinging on its surface.

It has been found that a 1% to 10% solution of the water soluble reaction products is satisfactory for impregnating purposes. After squeezing out the excess impregnating solution the fabric is dried at, for instance, about 60° C. for 15 to 20 minutes or at 100°-110° C. for 1 to 2 minutes in a current of air. By this treatment the fabric is thoroughly dried. It is then heated to a higher temperature of, for instance, 140°-145° C. for about 15 minutes or at 160°-165° C. for from 2 to 5 minutes, or even at 170° C. for 1 minute. This latter treatment fixes the fatty acid nitrile-fatty acid chloride-formaldehyde reaction product on the fabric, rendering it insoluble in water and organic solvents.

It has further been ascertained that certain metallic soaps may be incorporated in the impregnating solutions of the present invention to the extent of about 0.1% to 2% to enhance the initial water repellency of the treated fabrics. Although the fabrics do not retain the metallic soap to any substantial degree after dry clean-

ing, the effect appears to last through several standard soap and water washings.

The following examples are given to illustrate the process of the present invention. All proportions are in parts by weight.

Example 1.—A reaction product was formed by heating together 137.3 parts of palmityl chloride, 132.7 parts of stearonitrile, 22.5 parts of paraformaldehyde and 1.4 parts zinc chloride for 22½ hours at 77° C. followed by reaction with 40 parts of pyridine at 55° C. for 23 hours. Four parts of this material were dissolved in 20 parts of denatured alcohol and 74 parts of warm water (60° C.) containing 2 parts of sodium acetate trihydrate added. A somewhat cloudy soapy solution was formed. This solution was used to impregnate a cotton gabardine fabric which was then squeezed between rubber rollers to remove the excess of solution, dried at 80° C. for 5 minutes and baked at 145° C. for 15 minutes.

In order to test the water repellency of this fabric a cut off section was dry cleaned by tumbling it in a container with a dry cleaning fluid known to the trade as Stoddards solvent, for about 20 minutes at about 80° C. The sample was squeezed out, dried in the air and ironed smooth. To test the fastness to washing of the water repellent fabric, an electric washing machine was filled with ¼% aqueous neutral soap solution at 90°-100° C. and the fabric washed for 40 minutes. It was then rinsed thoroughly with water and ironed dry. The above two tests will hereinafter be referred to as a "standard dry clean" and "standard wash," respectively. In order to test the degree of repellency the cloth to be tested was fastened in a 6 inch metal embroidery hoop placed at a 45° angle under a 6 inch glass laboratory funnel to which was attached by a 2 inch rubber tube a spray nozzle. The bottom of the spray nozzle was 6 inches above the surface of the cloth and 250 cc. of water at 80° F. was allowed to flow through the nozzle onto the cloth sample. A rating of 100 was given if no water adhered to the cloth; 90 indicated slight spotting; 80 a surface wetting only where the water directly impinged, and 50 a surface wetting of 50% of the area covered by the spray.

The cotton gabardine was subjected to these tests and gave as an original reading 90, after standard washing 85, and after standard dry cleaning 75.

Example 2.—A reaction product was formed by heating 120.6 parts of lauromitrile, 145.6 parts of lauryl chloride, 40 parts of paraformaldehyde, and 2.5 parts of zinc chloride at 75°-80° C. for

23 hours followed by reaction with 52.6 parts of pyridine at 75° C. for 20 hours. A solution was formed by dissolving 10 parts of the above reaction product in 187 parts of warm water (60° C.) containing 3 parts of sodium acetate trihydrate. A cotton gabardine fabric was impregnated with the solution, squeezed between rubber rollers to remove excess solution, dried at 80° C. and baked at 145° C. for 15 minutes. An initial spray reading of 80 was obtained. After standard washing a reading of 85, and after standard dry cleaning a reading of 75 was secured.

*Example 3.*—A reaction product was prepared by heating 137.3 parts of a commercial mixture of fatty acid chlorides (which consists of 70% hexadecanoyl chloride, 25% octadecanoyl chloride and 5% unreacted fatty acids), 132.7 parts of stearonitrile, 30 parts of paraformaldehyde and 2.7 parts of zinc chloride at 77° C. for 21 hours, followed by reaction with 37.2 parts of alpha picoline and 7.9 parts of pyridine at 65°-70° C. for 21 hours. 173.9 parts of this reaction product were mixed while warm with an equal weight of dry dioxan and stirred vigorously while cooling. A homogeneous smooth paste was formed at room temperature. A solution was formed by mixing 40 parts of this paste with 354 parts of warm water (65° C.) containing 6.6 parts of sodium acetate trihydrate. This solution was used to impregnate cotton gabardine, a light brown dyed mercerized broadcloth having the designation 136 x 72 3.55 and an olive drab dyed mercerized poplin having the designation 102 x 56 2.25. All the cloths were squeezed free of excess solution between rubber rollers, and dried at 80°-90° C. for 10 minutes. They were then baked for varying lengths of time at 160° C. and cuttings given standard dry cleanings. The table below gives the results as obtained on the spray testing device.

| Sample                | Baking time | Initial reading | After standard dry clean |
|-----------------------|-------------|-----------------|--------------------------|
| <i>Minutes</i>        |             |                 |                          |
| Cotton gabardine..... | 4           | 100             | 95                       |
| Do.....               | 5           | 100             | 95                       |
| Do.....               | 10          | 100             | 95                       |
| Broadcloth.....       | 4           | 100             | 90                       |
| Do.....               | 5           | 100             | 90                       |
| Do.....               | 10          | 100             | 90                       |
| Poplin.....           | 4           | 95              | 85                       |
| Do.....               | 5           | 95              | 85                       |
| Do.....               | 10          | 95              | 85                       |

*Example 4.*—35 parts of the reaction product described in Example 3 consisting of mixed palmityl and stearyl chlorides, stearonitrile, paraformaldehyde, alpha picoline and pyridine (but no dioxan) were ground thoroughly with 12.5 parts of anhydrous sodium sulfate and 2.5 parts of aluminum distearate. When homogeneous 12 parts of dry dioxan were added to give a stiff paste. A solution was formed by dissolving 12 parts of the above paste in 10 parts of denatured alcohol and adding 175 parts of warm water (65° C.) containing 3 parts of sodium acetate trihydrate. Samples of mercerized poplin (102 x 56 2.25) and mercerized broadcloth (136 x 72 3.55) were impregnated with the solution, squeezed, dried and baked at 160° C. for 5 minutes. The initial spray readings on both the poplin and broadcloth were 100. After a standard dry cleaning the spray reading on the poplin was 85 and on the broadcloth, 90.

*Example 5.*—A slightly cloudy soapy solution

was made up by mixing 20 parts of the dioxan paste formed in Example 3 with 177 parts of water at 65° C. containing 3.3 parts of sodium acetate trihydrate. A sample of acetate silk fabric, woolen flannel and a silk stocking were impregnated with the solution, squeezed free of excess solution, dried at 70°-80° C. and baked at 160° C. for 5 minutes. Cuttings of these treated pieces were also given a standard dry cleaning. The spray readings obtained are given below.

| Sample             | Initial reading | Reading after standard dry clean |
|--------------------|-----------------|----------------------------------|
| Acetate silk.....  | 90              | 75                               |
| Flannel.....       | 100             | 95                               |
| Silk stocking..... | 100             | 95                               |

The above examples illustrate the preferred process of the present invention but many variations on the procedure may be made without departing from the spirit of the invention. It will also be seen that reaction products of acid chloride, nitrile, paraformaldehyde and tertiary amine, wherein the nitrile and acid chloride contain carbon chains of 15 or more carbon atoms yield the best water repellent effects on treated fabrics. However, in some cases those products containing carbon chains of less than 15 but more than 9 carbon atoms are very satisfactory and yield highly water repellent effects.

To note another instance, very excellent water repellent products may be made by utilizing reaction products of waxes with acid chloride-forming reagents such as the phosphorus chlorides and thionyl chloride in the products of my copending application Serial Number 392,937, filed May 10, 1941. Such waxes may include montan, candelilla, and the like. These reaction products may be substituted in whole or in part for the acid chlorides in the above products. When textile materials are treated with these wax compositions according to the process of the present invention excellent water repellence is secured with substantially no decrease in the tensile strength of the treated fabric. This is in accordance with the observation that the reaction products of acid chlorides, nitriles and paraformaldehyde in general when used in the process of the present invention do not seriously lower the tensile strength of the treated fabrics. Textile treating compositions prepared from waxes are described in an application of Raymond A. Pingree, Cranston, R. I., Serial No. 429,400, filed Feb. 3, 1942.

When employing metallic soaps in the process of the present invention it has been found that certain soaps are more satisfactory than others. Among those giving the best results are aluminum distearate, cerium stearate and lead stearate. Other soaps which have been used are aluminum monostearate, aluminum tristearate, barium stearate, aluminum palmitate, calcium stearate, magnesium stearate, strontium stearate and zinc stearate.

It has been ascertained that the process of the present invention may be more easily carried out by using a paste formed from the nitrile-acid chloride-formaldehyde-amine reaction products and an inert water-soluble solvent. Dioxan is inert and readily water-soluble and when thoroughly dried makes an excellent, readily water-dispersible paste with the aforementioned reaction products. However, other materials may

be employed such as the diethyl ether of diethylene glycol, methyl acetate, ethyl lactate, the mono methyl ether of diethylene glycol acetate and the like.

Although I have given several specific temperatures of drying and baking great variations may be made and higher or lower temperatures employed to secure desirable results.

What I claim is:

1. A process of making textile fabrics water repellent without seriously lowering the tensile strength thereof comprising impregnating a textile fabric with an aqueous solution of from 1% to 10% of a reaction product of a tertiary amine with the compound formed from the reaction of a nitrile containing a chain of more than 9 carbon atoms, an acid chloride containing a chain of more than 9 carbon atoms and formaldehyde, drying said impregnated textile fabric at below 110° C., and baking said dried impregnated textile fabric between 110° C. and 160° C. for from 1 to 15 minutes.

2. A process of making textile fabrics water repellent without seriously lowering the tensile strength thereof comprising impregnating a textile fabric with an aqueous solution containing 0.1% to 2% of a metallic soap and 1% to 10% of a reaction product of a tertiary amine with the compound formed from the reaction of a nitrile containing a chain of more than 9 carbon atoms, an acid chloride containing a chain of more than 9 carbon atoms and formaldehyde, drying said impregnated textile fabric at below 110° C., and baking said dried impregnated textile fabric between 110° C. and 160° C. for from 1 to 15 minutes.

3. A process of making textile fabrics water repellent without seriously lowering the tensile strength thereof comprising impregnating a textile fabric with an aqueous solution formed by mixing water with 2% to 20% of a paste consist-

ing of between 30% and 50% dioxan and between 70% and 50% of a reaction product of a tertiary amine with the compound formed from the reaction of a nitrile containing a chain of more than 9 carbon atoms, an acid chloride containing a chain of more than 9 carbon atoms and formaldehyde, drying said impregnated textile fabric at below 110° C., and baking said dried impregnated textile fabric between 110° C. and 160° C.

10 for from 1 to 15 minutes.

4. A process of making textile fabrics water repellent without seriously lowering the tensile strength thereof comprising impregnating a textile fabric with an aqueous solution containing 0.1% to 2% of aluminum distearate and 1% to 10% of a reaction product of a tertiary amine with the compound formed from the reaction of a nitrile containing a chain of more than 9 carbon atoms, an acid chloride containing a chain of more than 9 carbon atoms and formaldehyde, drying said impregnated textile fabric at below 110° C., and baking said dried impregnated textile fabric between 110° C. and 160° C. for from 1 to 15 minutes.

15 5. A process of making textile fabrics water repellent without seriously lowering the tensile strength thereof comprising impregnating a textile fabric with an aqueous solution formed by mixing water with 2% to 20% of a paste consisting of between 30% and 50% of an inert water-soluble solvent and between 70% and 50% of a reaction product of a tertiary amine with the compound formed from the reaction of a nitrile containing a chain of more than 9 carbon atoms, an acid chloride containing a chain of more than 9 carbon atoms and formaldehyde, drying said impregnated textile fabric at below 110° C., and baking said dried impregnated textile fabric between 110° C. and 160° C. for from 30 35 40 1 to 15 minutes.

JOHN B. RUST.